

July 21, 1936.

A. O. AUSTIN

2,048,047

INSULATION FOR ELECTRICAL APPARATUS

Original Filed March 5, 1931



INVENTOR  
Arthur O. Austin  
BY *Alpheus J. Crane*  
ATTORNEY

## UNITED STATES PATENT OFFICE

2,048,047

## INSULATION FOR ELECTRICAL APPARATUS

Arthur O. Austin, near Barberton, Ohio, assignor, by mesne assignments, to The Ohio Brass Company, Mansfield, Ohio, a corporation of New Jersey

Original application March 5, 1931, Serial No. 520,285, now Patent No. 1,981,716, dated November 20, 1934. Divided and this application February 2, 1933, Serial No. 654,836

## 18 Claims. (Cl. 175—41)

This invention relates to capacitance members and dielectric filling material therefor, and has for one of its objects the provision of dielectric material for capacitance couplings which will have a substantially constant specific inductive capacity.

A further object of the invention is to increase the specific inductive capacity of filling material for capacitance couplings.

10 A further object is to provide filling material for capacitance couplings which will be less affected by moisture than material heretofore used.

15 A further object is to provide means for overcoming the effect of changes in temperature on capacitance couplings.

A further object is to provide a device of the class named which shall be of improved construction and operation.

20 Other objects and advantages will appear from the following description.

The invention is exemplified by the combination and arrangement of parts shown in the accompanying drawing and described in the following specification, and it is more particularly pointed out in the appended claims.

25 This is a division of application Serial Number 520,285, filed March 5, 1931 now Patent No. 1,981,716, dated November 20, 1934.

In the drawing:

30 The figure is an elevation with parts in section of a bushing insulator having one embodiment of the present invention applied thereto.

In oil filled bushings, particularly those used for high voltage, there may be, at times, an appreciable volumetric change in the oil or insulating compound due to changes in temperature. This is particularly true in the case of bushings for transformers of a conservator type where the lower ends of the bushings are subjected to the hot oil on the inside of the transformer housing. Roof or entrance bushings and their contents may be heated to a very large extent by heat from the sun. As the oil or insulating compound in the bushing has a rather large volumetric expansion compared to the material forming the shell of the bushing, it is necessary to make provision for this variation in volumetric expansion either by the use of expansion reservoirs or expansion space in the bushing.

40 If the amount of oil can be reduced, the amount of space required for expansion in the bushing, or the size of the expansion reservoirs may be materially reduced, thereby reducing the cost and size of a bushing for a given performance.

45 In bushings in which a capacitance coupling is

used, it is important that the amount of oil or filling compound in the bushing be reduced to a minimum so that the electrical characteristics of the electrostatic coupling remain as nearly constant as possible.

5 It is well known that a filling medium such as transformer oil will take up water, which in turn will affect its specific inductive capacity materially. While an increase in the specific inductive capacity of the oil is produced when the oil takes up water, this may be an advantage insofar as the capacitance coupling is concerned but the presence of water in the oil lowers its dielectric strength and may interfere with the performance of the bushing, particularly if the bushing is subjected to very high voltages.

A change in the effective specific inductive capacity of the zones formed by the filling medium will of course change the characteristics of the capacitance coupling. This, as well as the effect of different temperatures, will tend to cause the capacitance coupling to vary, making it less suitable where accuracy is required over a considerable period of time. This applies particularly where a close regulation is required, and in cases where voltage or energy is supplied by capacitance couplings for relay operation, metering or other purposes.

20 In order to provide increased energy from the capacitance coupling, to reduce the volumetric change in the filling medium and to prevent change in the capacitance of the capacitance coupling caused by change in the specific inductive capacity of the filling medium when water is absorbed or lost by the filling medium, the present invention contemplates the use of a supplemental dielectric or filling medium which will reduce the quantity of the liquid filling medium in the zone affecting the dielectric strength and capacitance coupling. In general, this can be accomplished by filling the space largely with insulating baffles of material such as porcelain, glass or other substance which will not take up or lose water. For manufacturing reasons, however, it is difficult to fill with baffles all of the space between the metallic surfaces which have a difference in potential. It is generally advisable to allow some space between the parts to provide for irregularities, and also for an insulating medium which will provide insulation even in case some of the insulating sleeves or baffles are broken or damaged.

45 One method of improving the characteristics and the advantages outlined above is to fill the space between the baffles with a solid material

5

50

55

made up in small pieces. This will displace a large part of the liquid filling medium and at the same time the specific inductive capacity of the dielectric in the filled space may be materially increased, providing the solid filling material has a higher specific inductive capacity than the liquid filling medium displaced. The solid material used for filling may be sand, or pieces composed of glass, porcelain or other material which has a higher specific inductive capacity than the liquid filling medium displaced.

The specific inductive capacity of the material used for filling material can be utilized to distribute or control the stress in the various zones in the bushing. If a zone of high stress is filled in with material having a higher specific inductive capacity than the liquid dielectric displaced, the stress over this zone will be reduced. The filling material may therefore be used to control the distribution of stress in the bushing as well as to control the effective capacitance, and to reduce the amount of liquid filling material required for filling in the voids or interstices.

By using a filling material which has pore spaces, it is possible to fill the pore spaces with water or other medium which will materially increase its specific inductive capacity. At the same time the surrounding structure of solid material will tend to maintain the dielectric strength of the particles so that the effective insulation will not be materially interfered with.

As it is exceedingly difficult to remove water or other liquid from material which has very small pore spaces, a porous filling material will tend to retain its moisture and thereby maintain a more constant condition than a filling medium such as insulating oil, which will take up or give off moisture readily under changes in temperature and humidity of the air with which it is in contact.

It is also possible to use insulating baffles made of refractory or ceramic materials which have pore spaces. This material if filled with water and immersed in a liquid dielectric medium will have a very high effective insulation and an increased effective specific inductive capacity. It is therefore possible to use insulating baffles as well as granular material having an increased specific inductive capacity in zones of higher stress such as that adjacent to the center electrode in a bushing.

The reduction of stress upon this zone will transfer the electrical stress to other zones, thereby tending to equalize the electrical stress. In addition, the increase in effective capacitance of the zones subjected to the higher stress due to position will also increase the effective capacitance and, consequently, the output of the capacitance coupling.

One advantage of the filling material is that it tends to prevent a discharge under high static stress which would tend to drive away the oil where the electrode surfaces terminate. The filling material may also be used to control the surface gradient on the outside of the bushing to an appreciable extent where it is possible to fill zones in such a way that the path of electrostatic flux will be directed by the filling material.

Several means may be used to control the stability of the insulating baffles, and the filling material used. By using a material for baffles and filling having very small pore spaces the retention of moisture or liquid in the pores which will increase the effective specific inductive capacity will be such that there will be little tend-

ency to change the amount present. In some cases, however, where the pore spaces are relatively large, it may be necessary or advisable to cover the impregnated particles or baffles with a varnish, glaze or other material which will retain the entrapped moisture so it will not change with time. The insulating baffles may be glazed on one surface, which will seal the pores, and the unglazed surface, or openings left in the glaze for impregnating, may be covered with an insulating varnish or other material later. Very fine pore spaces may be equivalent to a pressure of several thousand pounds per square inch, in their effect on the retention of moisture, and if small openings are provided in the glaze, the material may be impregnated or largely saturated with water or other medium which will be retained even though conditions change materially. Where the pore spaces are larger, the impregnating may be materially accelerated by placing the whole under a high pressure in the liquid used for impregnating.

The drawing shows one form of the invention applied to a transformer, circuit breaker, metering or other bushing. The bushing has a central electrode or conductor 10 and a mounting flange 11. Insulating baffles 12 and 13 are placed between the supporting flange 11 and the conductor 10. The insulating baffles are surrounded by shells 14 and 15. The baffle 13 carries a sleeve 30 or zone 16 of conducting material insulated from the conductor 10 and the flange 11 and forming a capacitance coupling with the conductor 10. The primary 17 of a step-down transformer is connected by a lead 18 to the capacitance member 16, the other terminal of the transformer winding being grounded.

In order to improve the characteristics of the bushing and the capacitance coupling described above, the spaces 19, 20, 21, and 22 are filled with granular, solid, dielectric material having high specific inductive capacity as described above. In order to provide a grading effect, the material used in zone 19 may have a higher effective specific inductive capacity than the material used in the zone 20. The intervening space or interstices between the pieces of filling material can be filled with an insulating oil or compound of the necessary dielectric properties. The grading of the dielectric stress may have a material economic advantage in the construction of the bushing as a zone having a high stress under normal conditions may have a portion of the stress transferred to other zones by increasing the effective capacitance of the highly stressed zones by means of a filling having higher specific inductive capacity. One method would be to use a porous material in the inner zone 19, a non-porous material in 20 and oil in 21 and 22. The zones could of course be materially changed in size to meet the conditions of design. With this arrangement the zone 19 would have its capacitance increased through the absorption of moisture from the oil which would have but little or no effect upon the material in zone 20.

As vibration may tend to change the location of the various particles of the granular dielectric material and under some conditions may result in an increase in the mechanical stress set up between the parts, owing to unequal expansion and contraction, it may be desirable to retain the particles of filling material in a fixed position. This can be readily accomplished in one of several ways. One method is to coat the pieces of filling material with a varnish, oil or other me-

dium which can be used to stick the particles together after they have set a short time. This may be done by filling the bushing with the granular material and the binding material in liquid form 5 and then drawing off excess binding material and allowing the remainder to harden either by drying or by the application of heat.

Another method is to apply a suitable varnish or oil to the granular particles after they have 10 been impregnated with water and then allowing the varnish or oil to harden. The coated particles may then be handled in a manner similar to uncoated particles of filling material or sand. After the coated particles are in place in the bushing, the bushing with the filling material may be 15 heated sufficiently to cause the material to soften and bind the several particles together. This will retain the particles in position and, at the same time, seal the pores and retain the material affecting the specific inductive capacity of the particles. It, of course, is also possible to hold the insulating baffles in place in the outer shell by the coating material on the several particles so that special holding means may be dispensed with. 20 This is particularly true for some of the smaller size bushings in which the saving in cost will more than offset the ability readily to replace a part.

I claim:

30. 1. A filling for electrical apparatus comprising particles of solid dielectric material, a binder for holding said particles together, said binder consisting only of a layer of such thickness as will adhere to the particles when the binder is in a liquid state and free to flow away by gravity, and an insulating liquid filling the interstices between said particles.
35. 2. A condenser comprising, a pair of spaced conductor elements and a porous dielectric interposed between said element and insulating said elements from each other, said dielectric having the pores thereof filled with water.
40. 3. In a condenser or capacitance coupling, spaced conductor elements and a porous dielectric interposed between said elements, said dielectric having the pores thereof filled with water and at least a portion of the surface thereof covered with a coating to retain the water in said pores.
45. 4. Filling material for housings for electrical apparatus comprising an aggregate of small individual particles of porous porcelain having the pores thereof filled with a substance of higher specific inductive capacity than the material of said particles.
50. 5. A filling for housings for electrical apparatus comprising an aggregate formed of porous dielectric particles, the pores of said particles being filled with water, and an insulating liquid filling the interstices between said particles.
55. 6. A condenser or capacitance coupling comprising spaced conductor elements, and a solid dielectric baffle interposed between said elements and insulating said elements from each other, said baffle being porous and having the pores thereof filled with water.
60. 7. A condenser or electrostatic coupling comprising spaced conductor elements and a solid baffle interposed between said elements, said baffle being porous and having the pores thereof filled with water, a portion at least of the surface of said baffle being covered with coating material to retain the water in said pores.
70. 8. A filling for electrical apparatus comprising solid particles of porous dielectric material, water

filling the pores of said material, and a binder covering said particles to retain the water therein and to hold said particles together.

9. The combination with a bushing insulator having a capacitance coupling therein, of a filling for said insulator comprising an aggregate formed of particles of porous material, a binder disposed on the surfaces of said particles for holding said particles together and for closing the pores of said particles to retain in said pores any liquid 10 that may be therein, said binder being substantially restricted to a surface coating of said particles of such thickness only as will adhere to said particles when said binder is in a liquid state and free to flow away by gravity, and an insulating liquid filling the interstices between said particles. 15

10. A filler for electrical apparatus comprising particles of porous dielectric material, the pores of said material being filled with water, a binder 20 holding said particles together and covering the surfaces thereof to retain the water in said pores, and an insulating liquid filling the interstices between said particles.

11. The dielectric element of a condenser 25 formed of porous non-combustible dielectric material having the pores thereof filled with a liquid of higher specific inductive capacity than said dielectric material.

12. The dielectric element of a condenser comprising porous dielectric material having the pores thereof filled with water. 30

13. The dielectric element of a condenser comprising porous dielectric material having the pores thereof filled with water and at least a portion 35 of the surface of said material covered with a coating to retain the water in said pores.

14. A dielectric baffle for electrical apparatus comprising a plate formed of porous porcelain having a liquid in the pores of said porcelain of higher specific inductive capacity than said dielectric material. 40

15. The dielectric element of a condenser comprising a unitary porous plate of dielectric material having the pores thereof filled with water. 45

16. A dielectric baffle for a condenser comprising a unitary porous plate of dielectric material having the pores thereof filled with water and at least a portion of the surface of said plate covered with coating material to retain the water in said pores. 50

17. A dielectric filler for electrical apparatus comprising an aggregate formed of particles of porous material, a binder disposed on the surface of said particles for holding said particles together and for closing the pores of said particles to retain in said pores any liquid that may be therein, said binder being substantially restricted to a surface coating of said particles of such thickness only as will adhere to said particles when said binder is in a liquid state and free to flow away by gravity, and an insulating liquid filling the interstices between said particles. 55

18. A condenser or capacitance coupling comprising spaced conductor elements and a dielectric element interposed between said conductor elements and composed of porous porcelain having the pores thereof filled with a substantially non-conducting liquid having a higher specific inductive capacity than the porcelain of said dielectric element. 60

ARTHUR O. AUSTIN.